

Patented Dec. 26, 1944

2,366,042

# UNITED STATES PATENT OFFICE

2,366,042

## LUBRICANTS

John D. Morgan, South Orange, N. J., assignor to  
Cities Service Oil Company, New York, N. Y., a  
corporation of Pennsylvania

No Drawing. Application October 22, 1942,  
Serial No. 462,903

12 Claims. (Cl. 252—36)

This invention relates to lubricants and more particularly to a lubricant which is essentially a single chemical compound that has a comparatively uniform viscosity over a wide temperature range.

Petroleum lubricants are made up of a mixture of a large number of different hydrocarbons. There are generally paraffinic, aromatic and naphthenic hydrocarbons as well as some olefinic hydrocarbons in lubricants. It is very hard to control the physical properties of this mixture of hydrocarbons and to obtain a mixture of uniform composition which has uniform physical properties. The viscosities of petroleum lubricants vary quite widely with changes in temperature.

The primary object of the present invention is to provide a lubricant which has a comparatively uniform viscosity over a wide temperature range.

A further object of the invention is to provide a lubricant, the base of which is a synthetic compound having a fixed composition.

A further object of the invention is to provide a lubricant, the base of which is normal hexyl ether.

A further object of the invention is to provide a lubricant which is a synthetic compound and colloidally combined with a metallic soap.

Another object of the invention is to provide a lubricant, the base of which is a synthetic compound having a fixed composition and containing an addition agent to provide an increased load-carrying capacity and being non-corrosive to bearing metals.

With these and other objects in view the invention consists in the improved lubricant hereinafter described and particularly defined in the claims.

I have discovered that normal hexyl ether, a colorless liquid, is a viscous product containing oiliness characteristics and having good lubricating properties. Normal hexyl ether has better load-carrying capacity than a Pennsylvania neutral oil having a viscosity of 200 at 100° F. and with a small amount of extreme pressure additive agent, normal hexyl ether has high extreme pressure load-carrying characteristics.

Normal hexyl ether has a comparatively uniform viscosity over a comparatively wide temperature range. For example, the viscosity at minus 40° F. is 15 centistokes, the viscosity at zero degrees F. is 5.48 centistokes; at 100° F. the viscosity is 1.59 centistokes; and at 200° F. the viscosity is .86 centistokes. The freezing

point of normal hexyl ether is below 50 degrees below zero F.

Several extreme pressure additives are soluble in normal hexyl ether and give high load-carrying properties to normal hexyl ether as a lubricant. For example, Polane, a commercial product which is a chlorinated ester of a fatty acid, such as chloromethyl stearate, made according to Lincoln et al. Patent No. 1,944,941 is very effective. Santolube No. 261, a commercial product which is a metallic derivative of alkylated carboxylic acid containing tin and sulfur, the tin being 3.25% by weight and sulfur .8% by weight of the compound. Santolube No. 261 is 15 a sulfurized tin salt of an alkyl phenol carboxylic acid manufactured under Patents Nos. 2,197,834—5, 2,256,441, and 2,257,751. A sulfurized tricresyl phosphine made according to the disclosure of Engelke Patent No. 2,260,303, is an 20 excellent extreme pressure agent. The addition of from 3% to 1% of any of the above additives to normal hexyl ether will give extreme pressure load-carrying capacity to the normal hexyl ether so that when tested in a 4-ball testing machine there will be no seizure at a pressure of 1000 lbs. which is the limit of loading the testing machine.

Normal hexyl ether is colloidally miscible with lithium and aluminum soaps to provide a grease 30 which has a comparatively uniform viscosity over a wide temperature range. The soaps are preferably stearates, although oleates may be used. In making the grease, the soap is dissolved in the normal hexyl ether. From .3% to 35 1% by weight of one of the additives discussed above is added to the ether in order to make an extreme pressure load-carrying grease. It has been found that a hexyl ether grease will result when 83% to 92% of normal hexyl ether has colloidally dispersed therein from 6% to 12% of lithium soap and 1% to 3% of aluminum soap. It is desired furthermore to add to this mixture 1% to 2% of latex and .3% to 1% of Polane or Santolube No. 261, or a sulfurized tricresyl phosphine or other suitable extreme pressure agent.

The preferred form of the invention having been thus described what is claimed as new is:

1. A lubricant having comparatively uniform viscosity over a wide temperature range, consisting of normal hexyl ether having a small amount of an extreme pressure addition agent dissolved therein.

2. A lubricant having comparatively uniform viscosity over a wide temperature range, consisting of normal hexyl ether having from .3% to

1% of an extreme pressure addition agent dissolved therein.

3. A lubricant having a comparatively uniform viscosity over a wide temperature range, consisting essentially of normal hexyl ether having colloidally dissolved therein a sufficient proportion of a lithium soap to impart a grease consistency to the lubricant and a sufficient proportion of an extreme pressure agent to impart extreme pressure properties to the lubricant.

4. A lubricant having a comparatively uniform viscosity over a wide temperature range, consisting essentially of normal hexyl ether having colloidally dissolved therein a sufficient proportion of lithium stearate to impart a grease consistency to the lubricant and a sufficient proportion of an extreme pressure agent to impart extreme pressure properties to the lubricant.

5. A lubricant having comparatively uniform viscosity over a wide temperature range, consisting of normal hexyl ether 83% to 92%; lithium stearate 6% to 12%; aluminum stearate 1% to 3%; latex 1% to 2%.

6. A lubricant having comparatively uniform viscosity over a wide temperature range, comprising a normal hexyl ether 82% to 92%; lithium stearate 6% to 12%; aluminum stearate 1% to 3%; latex 1% to 2%; extreme pressure addition agent .3% to 1%.

7. A method of lubricating metal bearings, comprising applying to the bearing a lubricant consisting essentially of normal hexyl ether.

8. A method of lubricating metal bearings, comprising applying to the bearing a solution consisting essentially of normal hexyl ether having a small amount of an extreme pressure additive agent dissolved therein.

9. A method of lubricating metal bearings, comprising applying to the bearing a solution consisting essentially of normal hexyl ether having from .3% to 1% of an extreme pressure additive dissolved therein.

10. A method of lubricating bearings, comprising applying to the bearing to be lubricated a colloidal lubricant consisting essentially of normal hexyl ether having dissolved therein a proportion of lithium stearate sufficient to impart a grease consistency to the lubricant.

11. A lubricant comprising a major proportion of normal hexyl ether and a minor proportion of lithium and aluminum stearates, the aluminum stearate being present in smaller proportion than the lithium stearate, and said stearates being present in the lubricant in sufficient proportion to impart a grease consistency to the lubricant.

12. A lubricating grease, comprising from about 6% to about 12% of a lithium soap, the remainder of the grease consisting essentially of normal hexyl ether.

JOHN D. MORGAN.